

# United States Patent [19]

Hendricks et al.

[11] 4,294,579  
[45] \* Oct. 13, 1981

[54] **PROCESS FOR THE ONE-BATH,  
SINGLE-STAGE DYEING OR PRINTING OF  
CELLULOSE FIBRES WITH  
FIBRE-REACTIVE DISPERSE DYESTUFFS**

[75] Inventors: **Udo-Winifred Hendricks; Dietrich  
Hildebrand, both of Odenthal; Robert  
Kuth, Cologne, all of Fed. Rep. of  
Germany**

[73] Assignee: **Bayer Aktiengesellschaft,  
Leverkusen, Fed. Rep. of Germany**

[\*] Notice: The portion of the term of this patent  
subsequent to May 19, 1998, has been  
disclaimed.

[21] Appl. No.: **69,690**

[22] Filed: **Aug. 27, 1979**

## [30] Foreign Application Priority Data

Apr. 7, 1979 [DE] Fed. Rep. of Germany ..... 2914142

[51] Int. Cl.<sup>3</sup> ..... **D06P 3/66; D06P 3/84**

[52] U.S. Cl. ..... **8/549; 8/576;  
8/609; 8/918**

[58] Field of Search ..... **8/171, 54.2, 189, 84,  
8/93, 173, 79, 163, 188, 1 D, 1 E, 549, 576, 609,  
918**

## [56] References Cited

### U.S. PATENT DOCUMENTS

3,791,787 2/1974 Yamada et al. ..... 8/54.2

|           |         |                        |         |
|-----------|---------|------------------------|---------|
| 3,853,460 | 12/1974 | Balland .....          | 8/84    |
| 3,923,457 | 12/1975 | Ong et al. ....        | 8/93    |
| 3,945,793 | 3/1976  | Corbishuey et al. .... | 8/93    |
| 3,945,989 | 3/1976  | Angliker et al. ....   | 260/197 |
| 3,980,426 | 9/1976  | Feess et al. ....      | 81/173  |
| 4,115,053 | 9/1978  | Aeschlimann .....      | 8/163   |
| 4,149,849 | 4/1979  | Koch et al. ....       | 8/54.2  |

### FOREIGN PATENT DOCUMENTS

1530104 10/1970 United Kingdom

### OTHER PUBLICATIONS

Translation Japan Kokai 78-143784 Publ. 12-14-78,  
Nose et al. "Process of Dyeing Active Hydrogen-Containing Fibers".

Primary Examiner—John C. Bleutge  
Attorney, Agent, or Firm—Sprung, Felfe, Horn, Lynch  
& Kramer

[57]

### ABSTRACT

Padding liquors or printing pastes which contain at least one compound which is free from ionic groups and possesses one or more glycicyl radicals are used for the one-bath, single-stage dyeing and printing of textile sheet-like structures of cellulose fibres or fibre blends containing cellulose fibres with water-insoluble reactive disperse dyestuffs in the absence of alkalis or alkaline compounds.

3 Claims, No Drawings

PROCESS FOR THE ONE-BATH, SINGLE-STAGE  
DYEING OR PRINTING OF CELLULOSE FIBRES  
WITH FIBRE-REACTIVE DISPERSE DYESTUFFS

The invention relates to a one-bath, single-stage process for dyeing or printing cellulose fibres or textile sheet-like structures containing cellulose fibres with water-insoluble reactive dyestuffs in the absence of alkalis or alkaline compounds. The process is characterised in that padding liquors or printing pastes are used which contain at least one compound which is free from 10 ionic groups and possesses one or more glycidyl radicals, and which have a pH value of between 7.5 and 2.7, especially between 7.0 and 3.5. The compounds possessing glycidyl groups are preferably water-soluble compounds which are liquid at room temperature and have a boiling point of not less than 220° C.

Particular mention should be made of compounds 20 containing glycidyl groups, of the formula



(I)

wherein

Q denotes a radical of the formula



25

30

or  $-CH_2-$ , or the group

represents an o-phenylene radical.

Amongst the compounds of the formula I, those of the formula



(III)

Z denotes a monovalent to tetravalent aliphatic hydrocarbon radical which can be interrupted by S-atoms, a cycloaliphatic hydrocarbon radical, a saturated heterocyclic radical or the groups PO, 35  $R_1-CO-N<$ ,



40

R denotes hydrogen or alkyl, R<sub>1</sub> denotes alkyl, cycloalkyl, aryl or aralkyl,Y denotes a radical of the formula  $-CO-CH_2-CH_2-SO_2-CH_2-CH_2-$  or  $-CH_2-CH_2-$ ,

A denotes alkylene or arylene,

m denotes 0 or 1,

n denotes 0-10,

q denotes 0 or 1 and

p denotes 1-4.

q only represents zero if m and n are zero and the glycidyl radical is bonded to a hetero-atom of Z.

If p represents 2-4, the substituents Q are bonded to different atoms of Z.

The bridge member Y is preferably bonded to a nitrogen atom of Z.

The aliphatic and cycloaliphatic hydrocarbon radicals are in particular optionally branched radicals with up to 8 C atoms.

Preferred aliphatic radicals Z and preferred alkyl radicals R and R<sub>1</sub> are those with 1-5 carbon atoms.Preferred cycloaliphatic radicals Z and cycloalkyl radicals R<sub>1</sub> are the cyclopentyl and cyclohexyl radical.

Aryl and aralkyl in particular represent phenyl and benzyl respectively.

A for example represents a C<sub>2</sub>-C<sub>6</sub>-alkylene or a phenylene radical.

Examples of heterocyclic radicals Z are the 1,3,5-hexahydrotriazine radical or radicals of the formula



(II)

wherein

R<sub>2</sub> represents hydrogen or the R<sub>2</sub>'s conjointly represent oxygen,R<sub>3</sub> represents hydrogen or methyl and

B represents



25

30

or  $-CH_2-$ , or the group

represents an o-phenylene radical.

Amongst the compounds of the formula I, those of the formula



(III)

40

wherein Z<sub>1</sub> denotes a monovalent to tetravalent aliphatic hydrocarbon radical with 1-5 carbon atoms, and n and p have the abovementioned meaning, those of the formula

(IV)

45

wherein n has the abovementioned meaning, and those of the formula



(V)

50

wherein Z<sub>2</sub> denotes the 1,3,5-hexahydrotriazine radical or a radical of the formula II,Y<sub>1</sub> denotes  $-CO-CH_2-CH_2-$  or  $-SO_2-CH_2-$ p<sub>1</sub> denotes 1-3,n has the abovementioned meaning and the radical in square brackets is bonded to a nitrogen atom of Z<sub>2</sub> are preferred.

Examples of the compounds I are:



$n = 0-8$ , especially 1-6







the same number of parts of the compound of the formula



is used, a similar dyeing is obtained.

A similar dyeing is also obtained if instead of the compound of the formula



the same number of parts of the formula



is used.

#### EXAMPLE 2

A mixed fabric consisting of 67 parts of poly(ethylene glycol terephthalate) and 33 parts of cotton is padded with a padding liquor which contains 70 parts of the reactive disperse dyestuff II and 30 parts of the compound of the formula



in 900 parts of water. The pH value of the padding liquor is 5.0. The fabric is squeezed off to a weight increase of 70% and then subjected to a hot air treatment at 220° C. for one minute. Thereafter the fabric is rinsed cold for five minutes and warm for five minutes and is subsequently soaped at the boil for 10 minutes with a wash solution which contains 5 parts of a customary detergent, for example a paraffinsulphonate, per 1,000 parts, rinsed warm for five minutes and dried. A clear blue dyeing having good fastness characteristics and good matching-shade dyeing of the two fibre components is obtained.

If instead of the compound of the formula



the same number of parts of the compound of the formula



is used, a dyeing of equal strength is obtained.

#### EXAMPLE 3

15 A mixed fabric consisting of 67 parts of poly(ethylene glycol terephthalate) and 33 parts of cotton is printed with an aqueous printing paste which contains 60 parts of the reactive disperse dyestuff III, 450 parts of 4% 20 strength aqueous alginate thickener, 50 parts of the compound of the formula



25 and 50 parts of polyethylene glycol in 1,000 parts, dried for 1 minute at 130° C. and then subjected to a hot air treatment at 220° C. for one minute. After thorough rinsing with cold and warm water, the fabric is soaped at the boil for 20 minutes with a solution which contains 1 part of a commercial paraffinsulphonate and 0.5 part of sodium carbonate in 1,000 parts, rinsed with warm water and dried. A deep red print with good matching-shade dyeing of the two fibre components is obtained, 40 with excellent yield from the dyestuff.

#### EXAMPLE 4

45 A mixed fabric consisting of 67 parts of poly(ethylene glycol terephthalate) and 33 parts of cotton is printed with an aqueous printing paste which contains 40 parts of the reactive disperse dyestuff IV, 20 parts of the disperse dyestuff VI, 550 parts of a 4% strength aqueous alginate thickener and 50 parts of the compound of the formula



50 55 in 1,000 parts. The fabric is dried for two minutes at 80° C. and then treated for 1 minute with hot air at 220° C. After thorough rinsing with cold and warm water, the fabric is then soaped at the boil for 20 minutes with a solution which contains 1 part of a commercial paraffinsulphonate and 0.5 part of sodium carbonate in 1,000 parts, rinsed with clear water and dried. A deep red print with good matching-shade dyeing of the two fibre components is obtained, with excellent yield from the dyestuff.

#### EXAMPLE 5

65 A mixed fabric consisting of 67 parts of poly(ethylene glycol terephthalate) and 33 parts of cotton is padded

with a padding liquor which contains 30 parts of the reactive disperse dyestuff V, 20 parts of the disperse dyestuff VIII, 10 parts of the compound of the formula



and 50 parts of polyethylene glycol in 890 parts of water, dried for 1 minute at 130° C. and then subjected to a hot air treatment at 200° C. for one minute. After thorough rinsing with cold and warm water, the fabric is soaped at the boil for 20 minutes with a solution which contains 1 part of a commercial paraffinsulphonate and 0.5 part of sodium carbonate in 1,000 parts, rinsed with warm water and dried. A clear yellow dyeing with good matching-shade dyeing of the two fibre components is obtained, with excellent yield from the dyestuff.

#### EXAMPLE 6

A mixed fabric consisting of 50 parts of viscose staple and 50 parts of polyamide is printed with an aqueous printing paste which contains 40 parts of the reactive disperse dyestuff of the formula IX, 20 parts of the disperse dyestuff VI and 40 parts of the compound of the formula



in 1,000 parts. The fabric is dried for 2 minutes at 80° C. and then steamed for 15 minutes with superheated steam at 180° C. After thorough rinsing with cold and warm water, the fabric is soaped at the boil for 20 minutes with a solution which contains 1 part of a commercial paraffinsulphonate and 0.5 part of sodium carbonate in 1,000 parts, rinsed with clear water and dried. A golden yellow print with good matching-shade dyeing of the two fibre components is obtained, with excellent yield from the dyestuff.

